

Oct. 19, 1937.

C. BIRDSEYE

2,096,084

ORNAMENTAL LAMP BULB OR THE LIKE AND METHOD OF MAKING THE SAME

Filed Sept. 30, 1935



Inventor  
Clarence Birdseye  
by Fenway & Witter  
Attorneys

## UNITED STATES PATENT OFFICE

2,096,084

ORNAMENTAL LAMP BULB OR THE LIKE  
AND METHOD OF MAKING THE SAMEClarence Birdseye, Gloucester, Mass., assignor,  
by mesne assignments, to Birdseye Electric  
Corporation, Dover, Del., a corporation of Del-  
aware

Application September 30, 1935, Serial No. 42,777

7. Claims. (Cl. 41—22)

The invention relates to the ornamentation of electric lamp bulbs by forming thereon silvered and etched areas disposed in novel relation and formed in a novel manner. I have discovered that a highly ornamental and decorative appearance may be imparted to electric lamp bulbs or the like by applying a coating of metallic silver to the inside walls of the bulb, or to selected portions thereof, and etching or frosting the exterior of the bulb in an area opposite to or supplementing the area of the silver coating and shaped so as to form a clear figure in the glass through which the outer surface of the bright silver of the coating is exposed to view in contrast to the pearl color of the etched background.

One type of electric lamp to which my invention has an especially useful application is that in which the inner surface of the silver coating is utilized as a reflecting surface, as for example, in a lamp designed for indirect lighting and having its curved end silvered up to its line of maximum diameter. When illuminated the lower part of such a bulb is darkened by the inside silver coating which prevents the passage of light rays. It is that portion of the lamp that I propose to ornament by forming on the exterior thereof a pearl-colored etched surface defining bands or other figures of artistic outline in the clear glass of the bulb. The bright outer surface of the silver of the inside coating is thus exposed to view in attractive contrast to the exterior background surface and a desirable appearance imparted to the lamp bulb both when illuminated and when unilluminated and this is particularly advantageous since lamps of this type usually require no exterior reflecting fixture but are fully exposed to view. My invention is in no sense limited to this or to any particular type of lamp, but includes within its scope of lamps having an inside silver coating for reflecting light from a source within the lamp bulb and an etched exterior surface defining a clear figure exposing to view the outer surface of the silver coating fully protected within the glass of the bulb.

In another aspect, my invention consists in a novel process of making ornamental lamp bulbs, characterized by the steps of applying a metallic silver coating to the inside of the bulb and etching the outer surface thereof in an area defining an unetched or clear figure above or opposite to the silvered coating. The order of the steps is of secondary importance only, it being more convenient as a general thing to carry out the

step of applying the silver coating before the step of etching the exterior surface of the article. Any satisfactory process may be employed for carrying out the coating step by which a continuous coating of metallic silver of substantially uniform thickness is formed and permanently bonded to the glass. One such process is disclosed in the copending application of Pincus Deren, Serial No. 42,227, filed September 26, 1935, and I prefer to employ the method of that application in putting the present invention into practice. Accordingly it is proposed first chemically to clean the inside of the bulb; then to place therein a limited quantity of a silver-depositing solution and then subject the solution to a turbulent agitation while the silver is being precipitated to cause the formation of a coating of uniform thickness and to prevent settling of precipitate which may be formed in the solution against the glass of the bulb. Having formed a silver coating in this manner, its area may be defined by removing the surplus silver from those parts of the bulb which are to be clear glass at least for the time being.

The step of forming an etched or frosted exterior surface on the bulb may be effected by dipping the bulb in any suitable etching solution and a number of solutions satisfactory for this purpose may be purchased in the open market. In order to form the desired clear figure or figures in the etched surface it is proposed to attach temporarily to the exterior of the bulb a mask of the desired configuration and contour. The mask may be provided in any one of numerous ways. For example, in forming ornamental bands about the bulb in the etched surface, it is necessary only to stretch elastic bands about the bulb. Other conventional or artistic designs may be formed by temporarily cementing a paper shield to the exterior of the bulb or coating the same with paraffin and then working the paraffin coating into an artistic configuration. Having provided the mask in the manner preferred, the bulb may now be dipped into the etching solution, whereupon the unprotected portions of the immersed surface are etched or frosted and thereby acquire the pearl-colored appearance characteristic of this treatment. In the etching operation the area of contact may be limited if desired by temporarily attaching a shield to the bulb. For example, in bulbs designed for indirect lighting, it is found desirable to limit the frosted area, similarly as the reflecting area, to the line of maximum diameter of the bulb. This may be done by providing the bulb

with a circular shield, contacting with the bulb at the desired line, and shielding it from contact with the etching solution above this line.

The characteristics of the method of my invention and the features of the product herein disclosed will be best understood and appreciated from the following description of the manner in which the process is carried out in ornamenting lamp bulbs and illustrated in the accompanying drawing in which,—

Fig. 1 is a view in elevation of a bulb in process of having the inside silver coating applied thereto, part of the bulb being broken away.

Fig. 2 is a sectional view on an enlarged scale, 15 of a bulb in process of having superfluous silver removed from its walls.

Fig. 3 is a view in elevation illustrating a silvered bulb provided with a mask.

Fig. 4 is a similar view showing a bulb provided 20 with a different form of mask.

Fig. 5 is a view in elevation of the bulb of Fig. 3 in the etching or frosting step, and

Fig. 6 is a view in elevation of a finished bulb.

In Fig. 1 I have illustrated the silver-depositing step as carried out and more fully disclosed in the application of Pincus Deren above identified. As shown in this figure the bulb 10 is inverted and stoppered by means of a combined stopper and holder 12 including a compressible 25 elastic section 14 which is expanded into tight sealing engagement with the neck of the bulb after the latter has been partially filled with a silver-depositing solution 16. The bulb is placed in inverted position and subjected to a movement which has an up and down component, a component in a circular path, and a rotary component about its own axis, as indicated by the arrows in Fig. 1. The result of this movement is to cause the silver-depositing solution to swash 30 or whirl upwardly and across the upper curved end of the bulb 10. This movement is continued during the silver-depositing process with the result that a uniform coating of metallic silver is deposited upon the upper portion of the bulb, 45 firmly bonded to the glass and free of pin holes or other imperfections. In addition to insuring a coating of uniform thickness, the movement imparted to the bulb prevents the settling of any precipitate in the solution against the glass of 50 the bulb. This is to be avoided since contact of precipitate prevents a secure bond from forming between the silver and the glass.

Having deposited a silver coating in the manner above described, its area may now be confined if desired, to a definite configuration within the bulb. This step is suggested in Fig. 2 in which the bulb 10, having the inside silvered coating 18, as shown, is held in a horizontal position in a holder which includes a clamp 20 for engaging 60 the curved end of the bulb, and a hold-down member 22. A rotary tool 24, provided with pivotally mounted scraping members 27 is introduced to the proper point within the bulb 10, and then rotated at high speed, whereupon the members 27 expand centrifugally against the walls of the bulb and in their rotation remove the silvered coating up to the line determined by gage mechanism, not shown. In Fig. 2 the tool 24 is shown as having removed the surplus silver from the 70 walls of the bulb up to its line of maximum diameter.

Having produced and shaped the silvered coating in the manner above explained, the bulb is next temporarily provided with a mask 26 of any 75 desired or artistic design. As shown in Fig. 3 a

conventional leaf design 28 of paper or other sheet material is illustrated as temporarily cemented to the curved end of the bulb, opposite to the silvered coating 18. In Fig. 4 another bulb 11 having a silvered coating 18, is shown as provided with a mask comprising two elastic bands 28 which are stretched about the bulb in spaced relation, slightly below its line of maximum diameter.

Having provided the bulb with a mask of the character indicated, the etching or frosting operation is next carried out as suggested in Fig. 5. For this purpose the bulb 10 is first provided with a limiting shield 30 of rubber or other flexible material which, in this case, is placed about the bulb so as to coincide at its lower edge with the line of maximum diameter of the bulb and the limiting line of the silvered coating 18. Thus equipped and still provided with the mask 26, the bulb is immersed to the proper level in the receptacle 32 containing liquid etching solution 34 and is maintained in this position for a sufficient length of time to permit the solution to act fully upon the exposed portions of the glass. The etched bulb is then withdrawn from the solution 20 and rinsed and the mask 26 removed.

The finished bulb is shown in Fig. 6. Its lower portion up to the line of maximum diameter is uniformly coated with a frosted or etched surface of attractive pearl color. This surface however, 30 defines a clear figure 38 of the shape determined by the mask 26, and through this clear figure the bright silver of the coating 18 is exposed to view as an exterior reflecting surface in attractive contrast to the pearl colored background 38. It will be understood that had the bulb 11 of Fig. 4 been similarly treated, it would appear in finished form with an etched surface ornamented by two parallel bright bands of silver.

While I have described the ornamentation of 40 a bulb by etched areas inclosing a clear figure, it is within the scope of the invention to reverse the proportion of the etched and clear areas, that is, to include or enclose an etched area or configuration within the clear area, giving the effect of an etched figure upon a silver background. By carrying out the method in this manner it may be utilized in applying useful as well as ornamental markings to the bulb, and I have in mind particularly trade-mark designs 45 and voltage data. In forming such marking the shield or mask will cover the major portion of the bulb surface, restricting the etched area to the desired marking. For example, the bulb may be dipped in liquid paraffin and then the glass 50 exposed by forming the desired design in the paraffin, so that the etched configuration is limited to the area in which the paraffin has been removed.

I have specifically referred to silver as a metal 55 suitable for the reflecting coating, but contemplate that other metals may be employed within the scope of my invention. For example nickel or rhodium may be employed or chromium may be deposited upon a thin priming coat of silver 60 thus making a composite metallic coating.

Having thus described my invention, what I claim as new and desire to secure by Letters Patent of the United States is—

1. The process of making lamp bulbs or the 70 like, which consists in applying a metallic coating to the inside surface of a bulb to present an inwardly directed reflecting surface, and etching the outer surface of the bulb in an area defining an unetched figure through which the outer sur- 75

- face of said metallic coating is exposed as an exterior reflecting surface.
2. The process of making lamp bulbs or the like, which consists in applying an inside coating of metallic silver to a bulb to present an inwardly directed reflecting surface, removing the marginal portions of the coating to form a defined reflecting area, and then etching the outer surface of the bulb in an area bounded coincidently with the reflecting area and circumscribing a clear figure through which the outer surface of said silvered coating is exposed as an exterior reflecting surface.
3. The process of making lamp bulbs or the like, which consists in applying a coating of metallic silver to the inside of the bulb with its inner surface forming a reflector of definite area, temporarily applying a mask of selected shape to the outer surface of the bulb opposite to a portion of the silvered area, immersing the bulb in etching solution to a depth covering the masked areas, and then removing the mask to expose the outer surface of said reflector in a bright silver figure bounded by an etched area.
4. The process of making lamp bulbs or the like, which consists in applying an inside coating of metallic silver to the rounded end of a bulb with the inner surface of the coating forming a reflector extending approximately up to the line of maximum diameter of the bulb, temporarily securing a figured mask to the outer surface of the bulb opposite to said inside silver coating, and then dipping the rounded end of the bulb with said mask into an etching solution substantially up to its line of maximum diameter, thereby forming an etched area through which the outer surface of said reflector is exposed in a figured design.
5. A lamp bulb or the like, comprising a hollow glass body having a coating of reflecting metal presenting a continuous inner surface for reflecting light from a source within the bulb, and an etched outer surface configuration adjacent to a clear area through which the outer surface of said metal coating is exposed to view in an arbitrary design.
6. An ornamental lamp bulb or the like, comprising a hollow glass body having a continuous coating of metallic silver upon a definite area of its inside walls presenting an inner surface for reflecting light from a source within the bulb, and an etched area of substantially similar contour upon its outer walls defining a clear figure through which the bright outer surface of said silver coating is exposed as an exterior reflecting surface.
7. An ornamental lamp bulb having its rounded end silvered upon the inside approximately up to the line of its maximum diameter presenting an inner surface for reflecting light from a source within the bulb, and an outer etched surface substantially coincident therewith and defining a clear figure through which the bright outer surface of said silver is exposed as an exterior reflecting surface in contrast to the pearl-colored etched surface.

CLARENCE BIRDSEYE.